



US009689227B2

(12) **United States Patent**  
Fripp et al.

(10) Patent No.: US 9,689,227 B2  
(45) Date of Patent: Jun. 27, 2017

- (54) **METHODS OF ADJUSTING THE RATE OF GALVANIC CORROSION OF A WELLBORE ISOLATION DEVICE**

(71) Applicant: **HALLIBURTON ENERGY SERVICES, INC.**, Houston, TX (US)

(72) Inventors: **Michael L. Fripp**, Carrollton, TX (US)  
**Zachary R. Murphree**, Carrollton, TX (US); **Zachary W. Walton**, Carrollton, TX (US)

(73) Assignee: **HALLIBURTON ENERGY SERVICES, INC.**, Houston, TX (US)

(\*) Notice: Subject to any disclaimer, the term of the patent is extended or adjusted under 3 U.S.C. 154(b) by 200 days.

(21) Appl. No.: **14/199,965**

(65) **Prior Publication Data**

US 2014/0202712 A1 Jul. 24, 2014

### Related U.S. Application Data

- (63) Continuation-in-part of application No. 13/491,995, filed on Jun. 8, 2012, now Pat. No. 8,905,147, and a (Continued)

(51) **Int. Cl.**  
*E21B 33/12* (2006.01)

(52) **U.S. Cl.**  
CPC ..... *E21B 33/1208* (2013.01); *E21B 33/12*  
..... (2013.01)

(58) Field of Classification Search

Field of Classification Search  
CPC ..... E21B 29/00  
See application file for complete search history.

- the application for complete search history.

10

## References Cited

U.S. PATENT DOCUMENTS

- 3,876,471 A 4/1975 Jones  
 4,573,517 A 3/1986 Booth et al.  
 (Continued)

(Continued)

## FOREIGN PATENT DOCUMENTS

- CA 2857123 6/2016  
EP 2354436 A2 8/2011

(Continued)

#### OTHER PUBLICATIONS

International Search Report and Written Opinion date mailed Mar. 31, 2015; PCT International Application No. PCT/US2014/068438.  
(Continued)

*Primary Examiner* — Jennifer H Gay

*Assistant Examiner* — Steven MacDonald

(74) Attorney, Agent, or Firm — McGuireWoods LLP

## ABSTRACT

A wellbore isolation device comprises a first material and pieces of a second material, wherein the first material: is a metal or a metal alloy; forms a matrix of the portion of the wellbore isolation device; and partially or wholly dissolves when an electrically conductive path exists between the first material and the second material and at least a portion of the first and second materials are in contact with the electrolyte, wherein the pieces of the second material: are a metal or metal alloy; and are embedded within the matrix of the first material; wherein the first material and the second material form a galvanic couple and wherein the first material is the anode and the second material is the cathode of the couple. The isolation device can also include a bonding agent for bonding the pieces of the second material into the matrix of the first material.

## 21 Claims, 4 Drawing Sheets



## Related U.S. Application Data

continuation-in-part of application No. PCT/US2013/027531, filed on Feb. 23, 2013.

(56)

## References Cited

## U.S. PATENT DOCUMENTS

|                  |         |                   |
|------------------|---------|-------------------|
| 5,570,502 A      | 11/1996 | Sawtell et al.    |
| 5,578,255 A      | 11/1996 | Okuyama et al.    |
| 7,077,200 B1     | 7/2006  | Adnan et al.      |
| 7,350,582 B2     | 4/2008  | McKeachnie et al. |
| 7,699,101 B2     | 4/2010  | Fripp et al.      |
| 7,708,937 B2     | 5/2010  | Meng et al.       |
| 7,798,236 B2     | 9/2010  | McKeachnie et al. |
| 8,211,248 B2     | 7/2012  | Marya             |
| 8,413,727 B2     | 4/2013  | Holmes            |
| 8,424,610 B2     | 4/2013  | Newton et al.     |
| 8,573,295 B2     | 11/2013 | Johnson et al.    |
| 2004/0045715 A1  | 3/2004  | Stoesz et al.     |
| 2005/0205265 A1  | 9/2005  | Todd et al.       |
| 2007/0089877 A1  | 4/2007  | Corre et al.      |
| 2007/0107908 A1  | 5/2007  | Vaidya            |
| 2007/0181224 A1  | 8/2007  | Marya et al.      |
| 2008/0066924 A1  | 3/2008  | Xu                |
| 2008/0149351 A1  | 6/2008  | Marya et al.      |
| 2008/0175744 A1  | 7/2008  | Motegi et al.     |
| 2008/0249637 A1  | 10/2008 | Asgari            |
| 2009/0025940 A1  | 1/2009  | Rytlewski         |
| 2009/0101334 A1  | 4/2009  | Baser et al.      |
| 2010/0270031 A1  | 10/2010 | Patel             |
| 2010/0294510 A1  | 11/2010 | Holmes            |
| 2011/0132619 A1  | 6/2011  | Agrawal           |
| 2011/0132621 A1  | 6/2011  | Agrawal et al.    |
| 2011/0136707 A1  | 6/2011  | Xu et al.         |
| 2011/0186306 A1  | 8/2011  | Marya et al.      |
| 2012/0118583 A1  | 5/2012  | Johnson et al.    |
| 2012/0175109 A1  | 7/2012  | Richard           |
| 2012/0273229 A1* | 11/2012 | Xu .....          |
|                  |         | E21B 23/00        |
|                  |         | 166/376           |
| 2012/0318513 A1  | 12/2012 | Mazyar et al.     |
| 2013/0032357 A1  | 2/2013  | Mazyar et al.     |
| 2013/0081814 A1  | 4/2013  | Gaudette et al.   |
| 2013/0133897 A1  | 5/2013  | Baihly et al.     |
| 2013/0146302 A1* | 6/2013  | Gaudette .....    |
|                  |         | E21B 31/002       |
|                  |         | 166/376           |
| 2013/0153236 A1  | 6/2013  | Bishop            |
| 2013/0206425 A1  | 8/2013  | Mazyar et al.     |
| 2013/0209175 A1  | 8/2013  | Keyworth          |
| 2013/0240200 A1  | 9/2013  | Frazier           |
| 2013/0269932 A1  | 10/2013 | Dams et al.       |
| 2013/0327540 A1* | 12/2013 | Hamid .....       |
|                  |         | E21B 33/12        |
|                  |         | 166/376           |
| 2013/0333899 A1  | 12/2013 | Xu                |
| 2014/0027128 A1* | 1/2014  | Johnson .....     |
|                  |         | B22F 1/02         |
|                  |         | 166/376           |
| 2014/0196899 A1  | 7/2014  | Jordan et al.     |

## FOREIGN PATENT DOCUMENTS

|    |                |    |         |
|----|----------------|----|---------|
| EP | 21188437       | B1 | 3/2012  |
| WO | 2007141465     | A1 | 12/2007 |
| WO | WO 2011017047  | A1 | 2/2011  |
| WO | WO 2012/091984 | A2 | 7/2012  |
| WO | WO 2013019409  | A2 | 2/2013  |
| WO | WO2013089941   | A1 | 6/2013  |

## OTHER PUBLICATIONS

- International Written Opinion date mailed May 27, 2015; PCT International Application No. PCT/US2015/014981.
- International Search Report and Written Opinion date mailed May 19, 2015; PCT International Application No. PCT/US2015/014988.
- T.Tanski, Synergy effect of heat and surface treatment on properties of the Mg—Al—Zn cast alloys, Journal of Achievements in Materials and Manufacturing Engineering, Oct. 2012, p. 260-274, vol. 54, Issue 2, Silesian University of Technology, Gliwice, Poland.
- Degradable Casing Perforation Ball Sealers and Methods for Use in Well Treatment, IPCOM000215741D, Mar. 7, 2012. Available at: <http://priorartdatabase.com/PCOM/000215741>.
- Solu-Plugs—Delayed Frac Plugs, IPCOM000176055D, Nov. 3, 2008. Available at: <http://www.ip.com/pubview/PCOM000176055D>.
- European Patent Office, Communication, European extended search report, Application No. 13801386.7, May 30, 2016.
- Patent Office of the Cooperation Council for the Arab States of the Gulf, Examination Report, Application No. GC2013-24222, dated Aug. 18, 2016.
- Australian Patent Office, Patent Examination Report No. 1, Australian Application No. 2015248171, Sep. 6, 2016.
- Australian Government IP Australia; Patent Examination Report No. 2; Apr. 29, 2016.
- Australian Patent Office, Patent Examination Report No. 1, Australian Application No. 2014377594, Jul. 21, 2016.
- European Patent Office, Communication (extended European search report, European Application No. 14878579.3, Apr. 25, 2017.
- Australian Patent Office, Patent Exam Report No. 2, Australian Application No. 2014377594, Sep. 29, 2016.
- European Patent Office, Communication pursuant to Rules 161(2) and 162 EPC, European Application No. 14878579.3, Jun. 3, 2016.
- PCT, International Search Report and Written Opinion, PCT Application No. PCT/US2014/068372, Mar. 19, 2015.
- Australian Patent Office, Patent Exam Report No. 1, Australian Application No. 2014385212, Jul. 14, 2016.
- European Patent Office, Communication pursuant to Rules 161(2) and 162 EPC, European Application No. 14884707.2, Jun. 16, 2016.
- Australian Patent Office, Patent Exam Report No. 1, Australian Application No. 2014385213, Aug. 11, 2016.
- Australian Patent Office, Patent Exam Report No. 2, Australian Application No. 2014385213, Oct. 12, 2016.
- European Patent Office, Communication pursuant to Rules 161(2) and 162 EPC, European Application No. 14884808.8, Jun. 21, 2016.
- PCT, International Search Report and Written Opinion, PCT Application No. PCT/US2014/068442, Mar. 19, 2015.
- European Patent Office, Communication pursuant to Rules 161(2) and 162 EPC, European Application No. 15780083.0, Oct. 26, 2016.
- Canadian Intellectual Property Office, Office Action, Canadian Application No. 2,868,885, Jan. 20, 2016.
- Canadian Intellectual Property Office, Office Action, Canadian Application No. 2,868,885, Oct. 27, 2016.
- Patent Office of the Cooperation Council for the Arab States of the Gulf, Examination Report, GC Application No. 2013-24222, May 11, 2016.
- PCT, International Search Report and Written Opinion, PCT Application No. PCT/US2013/027531, Dec. 9, 2014.

\* cited by examiner



FIG. 1



FIG. 2



FIG. 3



FIG. 4



FIG. 5



## METHODS OF ADJUSTING THE RATE OF GALVANIC CORROSION OF A WELLBORE ISOLATION DEVICE

### TECHNICAL FIELD

An isolation device and methods of removing the isolation device are provided. The isolation device includes at least a first material that is capable of dissolving via galvanic corrosion when an electrically conductive path exists between the first material and a different metal or metal alloy in the presence of an electrolyte. According to an embodiment, the isolation device is used in an oil or gas well operation. Several factors can be adjusted to control the rate of dissolution of the first material in a desired amount of time.

### BRIEF DESCRIPTION OF THE FIGURES

The features and advantages of certain embodiments will be more readily appreciated when considered in conjunction with the accompanying figures. The figures are not to be construed as limiting any of the preferred embodiments.

FIG. 1 depicts a well system containing more than one isolation device.

FIG. 2 depicts an isolation device according to an embodiment.

FIG. 3 depicts an isolation device containing a first, second, and third material according to another embodiment.

FIG. 4 illustrates wherein the third material bonds together the pieces of the first and second materials.

FIG. 5 illustrates wherein the third material is coated onto the pieces of the first and second materials.

FIG. 6 illustrates wherein the third material is a bonding agent for bonding the pieces of the second material into the matrix of the first material.

### DETAILED DESCRIPTION

As used herein, the words "comprise," "have," "include," and all grammatical variations thereof are each intended to have an open, non-limiting meaning that does not exclude additional elements or steps.

It should be understood that, as used herein, "first," "second," "third," etc., are arbitrarily assigned and are merely intended to differentiate between two or more materials, isolation devices, wellbore intervals, etc., as the case may be, and does not indicate any particular orientation or sequence. Furthermore, it is to be understood that the mere use of the term "first" does not require that there be any "second," and the mere use of the term "second" does not require that there be any "third," etc.

As used herein, a "fluid" is a substance having a continuous phase that tends to flow and to conform to the outline of its container when the substance is tested at a temperature of 71° F. (22° C.) and a pressure of one atmosphere "atm" (0.1 megapascals "MPa"). A fluid can be a liquid or gas.

Oil and gas hydrocarbons are naturally occurring in some subterranean formations. In the oil and gas industry, a subterranean formation containing oil or gas is referred to as a reservoir. A reservoir may be located under land or off shore. Reservoirs are typically located in the range of a few hundred feet (shallow reservoirs) to a few tens of thousands of feet (ultra-deep reservoirs). In order to produce oil or gas, a wellbore is drilled into a reservoir or adjacent to a reservoir. The oil, gas, or water produced from a reservoir is called a reservoir fluid.

A well can include, without limitation, an oil, gas, or water production well, or an injection well. As used herein, a "well" includes at least one wellbore. A wellbore can include vertical, inclined, and horizontal portions, and it can be straight, curved, or branched. As used herein, the term "wellbore" includes any cased, and any uncased, open-hole portion of the wellbore. A near-wellbore region is the subterranean material and rock of the subterranean formation surrounding the wellbore. As used herein, a "well" also includes the near-wellbore region. The near-wellbore region is generally considered to be the region within approximately 100 feet radially of the wellbore. As used herein, "into a well" means and includes into any portion of the well, including into the wellbore or into the near-wellbore region via the wellbore.

A portion of a wellbore may be an open hole or cased hole. In an open-hole wellbore portion, a tubing string may be placed into the wellbore. The tubing string allows fluids to be introduced into or flowed from a remote portion of the wellbore. In a cased-hole wellbore portion, a casing is placed into the wellbore that can also contain a tubing string. A wellbore can contain an annulus. Examples of an annulus include, but are not limited to: the space between the wellbore and the outside of a tubing string in an open-hole wellbore; the space between the wellbore and the outside of a casing in a cased-hole wellbore; and the space between the inside of a casing and the outside of a tubing string in a cased-hole wellbore.

It is not uncommon for a wellbore to extend several hundreds of feet or several thousands of feet into a subterranean formation. The subterranean formation can have different zones. A zone is an interval of rock differentiated from surrounding rocks on the basis of its fossil content or other features, such as faults or fractures. For example, one zone can have a higher permeability compared to another zone. It is often desirable to treat one or more locations within multiple zones of a formation. One or more zones of the formation can be isolated within the wellbore via the use of an isolation device to create multiple wellbore intervals. At least one wellbore interval corresponds to a formation zone. The isolation device can be used for zonal isolation and functions to block fluid flow within a tubular, such as a tubing string, or within an annulus. The blockage of fluid flow prevents the fluid from flowing across the isolation device in any direction and isolates the zone of interest. In this manner, treatment techniques can be performed within the zone of interest.

Common isolation devices include, but are not limited to, a ball and a seat, a bridge plug, a packer, a plug, and wiper plug. It is to be understood that reference to a "ball" is not meant to limit the geometric shape of the ball to spherical, but rather is meant to include any device that is capable of engaging with a seat. A "ball" can be spherical in shape, but can also be a dart, a bar, or any other shape. Zonal isolation can be accomplished via a ball and seat by dropping or flowing the ball from the wellhead onto the seat that is located within the wellbore. The ball engages with the seat, and the seal created by this engagement prevents fluid communication into other wellbore intervals downstream of the ball and seat. As used herein, the relative term "downstream" means at a location further away from a wellhead. In order to treat more than one zone using a ball and seat, the wellbore can contain more than one ball seat. For example, a seat can be located within each wellbore interval. Generally, the inner diameter (I.D.) of the ball seats is different for each zone. For example, the I.D. of the ball seats sequentially decreases at each zone, moving from the wellhead to

the bottom of the well. In this manner, a smaller ball is first dropped into a first wellbore interval that is the farthest downstream; the corresponding zone is treated; a slightly larger ball is then dropped into another wellbore interval that is located upstream of the first wellbore interval; that corresponding zone is then treated; and the process continues in this fashion—moving upstream along the wellbore—until all the desired zones have been treated. As used herein, the relative term “upstream” means at a location closer to the wellhead.

A bridge plug is composed primarily of slips, a plug mandrel, and a rubber sealing element. A bridge plug can be introduced into a wellbore and the sealing element can be caused to block fluid flow into downstream intervals. A packer generally consists of a sealing device, a holding or setting device, and an inside passage for fluids. A packer can be used to block fluid flow through the annulus located between the outside of a tubular and the wall of the wellbore or inside of a casing.

Isolation devices can be classified as permanent or retrievable. While permanent isolation devices are generally designed to remain in the wellbore after use, retrievable devices are capable of being removed after use. It is often desirable to use a retrievable isolation device in order to restore fluid communication between one or more wellbore intervals. Traditionally, isolation devices are retrieved by inserting a retrieval tool into the wellbore, wherein the retrieval tool engages with the isolation device, attaches to the isolation device, and the isolation device is then removed from the wellbore. Another way to remove an isolation device from the wellbore is to mill at least a portion of the device or the entire device. Yet, another way to remove an isolation device is to contact the device with a solvent, such as an acid, thus dissolving all or a portion of the device.

However, some of the disadvantages to using traditional methods to remove a retrievable isolation device include: it can be difficult and time consuming to use a retrieval tool; milling can be time consuming and costly; and premature dissolution of the isolation device can occur. For example, premature dissolution can occur if acidic fluids are used in the well prior to the time at which it is desired to dissolve the isolation device.

A novel method of removing an isolation device includes using galvanic corrosion to dissolve at least a portion of the isolation device. The rate of corrosion can be adjusted by selecting the materials used, the electrolyte used, the concentration of free ions available in the electrolyte, and the distance between the two materials of the galvanic system.

Galvanic corrosion occurs when two different metals or metal alloys are in electrical connectivity with each other and both are in contact with an electrolyte. As used herein, the phrase “electrical connectivity” means that the two different metals or metal alloys are either touching or in close enough proximity to each other such that when the two different metals are in contact with an electrolyte, the electrolyte becomes electrically conductive and ion migration occurs between one of the metals and the other metal, and is not meant to require an actual physical connection between the two different metals, for example, via a metal wire. It is to be understood that as used herein, the term “metal” is meant to include pure metals and also metal alloys without the need to continually specify that the metal can also be a metal alloy. Moreover, the use of the phrase “metal or metal alloy” in one sentence or paragraph does not mean that the mere use of the word “metal” in another sentence or paragraph is meant to exclude a metal alloy. As used herein, the term “metal alloy” means a mixture of two or more

elements, wherein at least one of the elements is a metal. The other element(s) can be a non-metal or a different metal. An example of a metal and non-metal alloy is steel, comprising the metal element iron and the non-metal element carbon.

5 An example of a metal and metal alloy is bronze, comprising the metallic elements copper and tin.

The metal that is less noble, compared to the other metal, will dissolve in the electrolyte. The less noble metal is often referred to as the anode, and the more noble metal is often 10 referred to as the cathode. Galvanic corrosion is an electrochemical process whereby free ions in the electrolyte make the electrolyte electrically conductive, thereby providing a means for ion migration from the anode to the cathode—resulting in deposition formed on the cathode. Metals can be 15 arranged in a galvanic series. The galvanic series lists metals in order of the most noble to the least noble. An anodic index lists the electrochemical voltage (V) that develops between a metal and a standard reference electrode (gold (Au)) in a given electrolyte. The actual electrolyte used can affect 20 where a particular metal or metal alloy appears on the galvanic series and can also affect the electrochemical voltage. For example, the dissolved oxygen content in the electrolyte can dictate where the metal or metal alloy appears on the galvanic series and the metal’s electrochemical 25 voltage. The anodic index of gold is -0 V; while the anodic index of beryllium is -1.85 V. A metal that has an anodic index greater than another metal is more noble than the other metal and will function as the cathode. Conversely, the metal that has an anodic index less than another metal is 30 less noble and functions as the anode. In order to determine the relative voltage between two different metals, the anodic index of the lesser noble metal is subtracted from the other metal’s anodic index, resulting in a positive value.

There are several factors that can affect the rate of 35 galvanic corrosion. One of the factors is the distance separating the metals on the galvanic series chart or the difference between the anodic indices of the metals. For example, beryllium is one of the last metals listed at the least noble end of the galvanic series and platinum is one of the first 40 metals listed at the most noble end of the series. By contrast, tin is listed directly above lead on the galvanic series. Using the anodic index of metals, the difference between the anodic index of gold and beryllium is 1.85 V; whereas, the difference between tin and lead is 0.05 V. This means that 45 galvanic corrosion will occur at a much faster rate for magnesium or beryllium and gold compared to lead and tin.

The following is a partial galvanic series chart using a deoxygenated sodium chloride water solution as the electrolyte. The metals are listed in descending order from the most noble (cathodic) to the least noble (anodic). The following list is not exhaustive, and one of ordinary skill in the art is able to find where a specific metal or metal alloy is listed on a galvanic series in a given electrolyte.

55 PLATINUM

GOLD

ZIRCONIUM

GRAPHITE

SILVER

CHROME IRON

SILVER SOLDER

60 COPPER-NICKEL ALLOY 80-20

COPPER-NICKEL ALLOY 90-10

MANGANESE BRONZE (CA 675), TIN BRONZE (CA903, 905)

65 COPPER (CA102)

BRASSES

NICKEL (ACTIVE)

TIN  
LEAD  
ALUMINUM BRONZE  
STAINLESS STEEL  
CHROME IRON  
MILD STEEL (1018), WROUGHT IRON  
ALUMINUM 2117, 2017, 2024  
CADMIUM  
ALUMINUM 5052, 3004, 3003, 1100, 6053  
ZINC  
MAGNESIUM  
BERYLLIUM

The following is a partial anodic index listing the voltage of a listed metal against a standard reference electrode (gold) using a deoxygenated sodium chloride water solution as the electrolyte. The metals are listed in descending order from the greatest voltage (most cathodic) to the least voltage (most anodic). The following list is not exhaustive, and one of ordinary skill in the art is able to find the anodic index of a specific metal or metal alloy in a given electrolyte.

| Anodic index                                                                                                                     |           |
|----------------------------------------------------------------------------------------------------------------------------------|-----------|
| Metal                                                                                                                            | Index (V) |
| Gold, solid and plated, Gold-platinum alloy                                                                                      | -0.00     |
| Rhodium plated on silver-plated copper                                                                                           | -0.05     |
| Silver, solid or plated; monel metal. High nickel-copper alloys                                                                  | -0.15     |
| Nickel, solid or plated, titanium and alloys, Monel                                                                              | -0.30     |
| Copper, solid or plated; low brasses or bronzes; silver solder; German silver; high copper-nickel alloys; nickel-chromium alloys | -0.35     |
| Brass and bronzes                                                                                                                | -0.40     |
| High brasses and bronzes                                                                                                         | -0.45     |
| 18% chromium type corrosion-resistant steels                                                                                     | -0.50     |
| Chromium plated; tin plated; 12% chromium type corrosion-resistant steels                                                        | -0.60     |
| Tin-plate; tin-lead solder                                                                                                       | -0.65     |
| Lead, solid or plated; high lead alloys                                                                                          | -0.70     |
| 2000 series wrought aluminum                                                                                                     | -0.75     |
| Iron, wrought, gray or malleable, plain carbon and low alloy steels                                                              | -0.85     |
| Aluminum, wrought alloys other than 2000 series aluminum, cast alloys of the silicon type                                        | -0.90     |
| Aluminum, cast alloys other than silicon type, cadmium, plated and chromate                                                      | -0.95     |
| Hot-dip-zinc plate; galvanized steel                                                                                             | -1.20     |
| Zinc, wrought; zinc-base die-casting alloys; zinc plated                                                                         | -1.25     |
| Magnesium & magnesium-base alloys, cast or wrought                                                                               | -1.75     |
| Beryllium                                                                                                                        | -1.85     |

Another factor that can affect the rate of galvanic corrosion is the temperature and concentration of the electrolyte. The higher the temperature and concentration of the electrolyte, the faster the rate of corrosion. Yet another factor that can affect the rate of galvanic corrosion is the total amount of surface area of the least noble (anodic metal). The greater the surface area of the anode that can come in contact with the electrolyte, the faster the rate of corrosion. The cross-sectional size of the anodic metal pieces can be decreased in order to increase the total amount of surface area per total volume of the material. The anodic metal or metal alloy can also be a matrix in which pieces of cathode material is embedded in the anode matrix. Yet another factor that can affect the rate of galvanic corrosion is the ambient pressure. Depending on the electrolyte chemistry and the two metals, the corrosion rate can be slower at higher pressures than at lower pressures if gaseous components are generated. Yet another factor that can affect the rate of

galvanic corrosion is the physical distance between the two different metal and/or metal alloys of the galvanic system.

According to an embodiment, a method of removing a wellbore isolation device comprises: contacting or allowing 5 the wellbore isolation device to come in contact with an electrolyte, wherein at least a portion of the wellbore isolation device comprises a first material and pieces of a second material, wherein the first material: (A) is a metal or a metal alloy; (B) forms a matrix of the portion of the wellbore 10 isolation device; and (C) partially or wholly dissolves when an electrically conductive path exists between the first material and the second material and at least a portion of the first and second materials are in contact with the electrolyte, wherein the pieces of the second material: (A) are a metal or 15 metal alloy; and (B) are embedded within the matrix of the first material; wherein the first material and the second material form a galvanic couple and wherein the first material is the anode and the second material is the cathode of the couple; and allowing at least a portion of the first material to 20 dissolve.

According to another embodiment, a method of removing a wellbore isolation device comprises: contacting or allowing the wellbore isolation device to come in contact with an electrolyte, wherein at least a portion of the wellbore isolation 25 device comprises pieces of a first material, pieces of a second material, and a third material, wherein the first material: (A) is a metal or a metal alloy; and (B) partially or wholly dissolves when an electrically conductive path exists between the first material and the second material and at 30 least a portion of the first and second materials are in contact with the electrolyte, wherein the second material is a metal or metal alloy, wherein the first material and the second material form a galvanic couple and wherein the first material is the anode and the second material is the cathode of the 35 couple, and wherein the third material physically separates at least a portion of a surface of one or more pieces of the first material from at least a portion of a surface of one or more pieces of the second material; and allowing at least some of the pieces of the first material to dissolve.

40 Any discussion of the embodiments regarding the isolation device or any component related to the isolation device (e.g., the electrolyte) is intended to apply to all of the method embodiments.

Turning to the Figures, FIG. 1 depicts a well system 10. 45 The well system 10 can include at least one wellbore 11. The wellbore 11 can penetrate a subterranean formation 20. The subterranean formation 20 can be a portion of a reservoir or adjacent to a reservoir. The wellbore 11 can include a casing 12. The wellbore 11 can include only a generally vertical wellbore section or can include only a generally horizontal wellbore section. A tubing string 15 can be installed in the wellbore 11. The well system 10 can comprise at least a first wellbore interval 13 and a second wellbore interval 14. The well system 10 can also include more than two wellbore 50 intervals, for example, the well system 10 can further include a third wellbore interval, a fourth wellbore interval, and so on. At least one wellbore interval can correspond to a zone of the subterranean formation 20. The well system 10 can further include one or more packers 18. The packers 18 can be used in addition to the isolation device to create the wellbore interval and isolate each zone of the subterranean formation 20. The isolation device can be the packers 18. The packers 18 can be used to prevent fluid flow between one or more wellbore intervals (e.g., between the first wellbore interval 13 and the second wellbore interval 14) via 55 an annulus 19. The tubing string 15 can also include one or more ports 17. One or more ports 17 can be located in each 60 65

wellbore interval. Moreover, not every wellbore interval needs to include one or more ports **17**. For example, the first wellbore interval **13** can include one or more ports **17**, while the second wellbore interval **14** does not contain a port. In this manner, fluid flow into the annulus **19** for a particular wellbore interval can be selected based on the specific oil or gas operation.

It should be noted that the well system **10** is illustrated in the drawings and is described herein as merely one example of a wide variety of well systems in which the principles of this disclosure can be utilized. It should be clearly understood that the principles of this disclosure are not limited to any of the details of the well system **10**, or components thereof, depicted in the drawings or described herein. Furthermore, the well system **10** can include other components not depicted in the drawing. For example, the well system **10** can further include a well screen. By way of another example, cement may be used instead of packers **18** to aid the isolation device in providing zonal isolation. Cement may also be used in addition to packers **18**.

According to an embodiment, the isolation device is capable of restricting or preventing fluid flow between a first wellbore interval **13** and a second wellbore interval **14**. The first wellbore interval **13** can be located upstream or downstream of the second wellbore interval **14**. In this manner, depending on the oil or gas operation, fluid is restricted or prevented from flowing downstream or upstream into the second wellbore interval **14**. Examples of isolation devices capable of restricting or preventing fluid flow between zones include, but are not limited to, a ball and seat, a plug, a bridge plug, a wiper plug, a packer, and a plug in a base pipe. A detailed discussion of using a plug in a base pipe can be found in U.S. Pat. No. 7,699,101 issued to Michael L. Fripp, Haoyue Zhang, Luke W. Holderman, Deborah Fripp, Ashok K. Santra, Anindya Ghosh on Apr. 20, 2010 and is incorporated herein in its entirety for all purposes. If there is any conflict in the usage of a word or phrase herein and any paper incorporated by reference, the definitions contained herein control. The portion of the isolation device that includes at least the first material and the second material can be the mandrel of a packer or plug, a spacer ring, a slip, a wedge, a retainer ring, an extrusion limiter or backup shoe, a mule shoe, a ball, a flapper, a ball seat, a sleeve, or any other downhole tool or component of a downhole tool used for zonal isolation.

As depicted in the drawings, the isolation device can be a ball **30** (e.g., a first ball **31** or a second ball **32**) and a seat **40** (e.g., a first seat **41** or a second seat **42**). The ball **30** can engage the seat **40**. The seat **40** can be located on the inside of a tubing string **15**. The inner diameter (I.D.) of the first seat **41** can be less than the I.D. of the second seat **42**. In this manner, a first ball **31** can be dropped or flowed into wellbore. The first ball **31** can have a smaller outer diameter (O.D.) than the second ball **32**. The first ball **31** can engage the first seat **41**. Fluid can now be temporarily restricted or prevented from flowing into any wellbore intervals located downstream of the first wellbore interval **13**. In the event it is desirable to temporarily restrict or prevent fluid flow into any wellbore intervals located downstream of the second wellbore interval **14**, then the second ball **32** can be dropped or flowed into the wellbore and will be prevented from falling past the second seat **42** because the second ball **32** has a larger O.D. than the I.D. of the second seat **42**. The second ball **32** can engage the second seat **42**. The ball (whether it be a first ball **31** or a second ball **32**) can engage a sliding sleeve **16** during placement. This engagement with the sliding sleeve **16** can cause the sliding sleeve to move; thus,

opening a port **17** located adjacent to the seat. The port **17** can also be opened via a variety of other mechanisms instead of a ball. The use of other mechanisms may be advantageous when the isolation device is not a ball. After placement of the isolation device, fluid can be flowed from, or into, the subterranean formation **20** via one or more opened ports **17** located within a particular wellbore interval. As such, a fluid can be produced from the subterranean formation **20** or injected into the formation.

Referring to FIGS. 2-3, the isolation device comprises at least a first material **51**, wherein the first material partially or wholly dissolves when an electrically conductive path exists between the first material **51** and a second material **52**. The first material **51** and the second material **52** are metals or metal alloys. The metal or metal alloy can be selected from the group consisting of, lithium, sodium, potassium, rubidium, cesium, beryllium, calcium, strontium, barium, radium, aluminum, gallium, indium, tin, thallium, lead, bismuth, scandium, titanium, vanadium, chromium, manganese, thorium, iron, cobalt, nickel, copper, zinc, yttrium, zirconium, niobium, molybdenum, ruthenium, rhodium, palladium, praseodymium, silver, cadmium, lanthanum, hafnium, tantalum, tungsten, terbium, rhenium, osmium, iridium, platinum, gold, neodymium, gadolinium, erbium, oxides of any of the foregoing, graphite, carbon, silicon, boron nitride, and any combinations thereof. Preferably, the metal or metal alloy is selected from the group consisting of magnesium, aluminum, zinc, beryllium, tin, iron, nickel, copper, oxides of any of the foregoing, and combinations thereof. According to an embodiment, the metal is neither radioactive, nor unstable.

According to an embodiment, the first material **51** and the second material **52** are different metals or metal alloys. By way of example, the first material **51** can be magnesium and the second material **52** can be iron. Furthermore, the first material **51** can be a metal and the second material **52** can be a metal alloy. The first material **51** and the second material **52** can be a metal and the first and second material can be a metal alloy. The first material and the second material form a galvanic couple and wherein the first material is the anode and the second material is the cathode of the couple. Stated another way, the second material **52** is more noble than the first material **51**. In this manner, the first material **51** (acting as the anode) partially or wholly dissolves when in electrical connectivity with the second material **52** and when the first and second materials are in contact with the electrolyte.

The methods include allowing at least a portion of the first material or at least some of the pieces of the first material to dissolve. The step of allowing can be performed after the step of contacting or allowing the first material to come in contact with the electrolyte. At least a portion of the first material **51** can dissolve in a desired amount of time. The desired amount of time can be pre-determined, based in part, on the specific oil or gas well operation to be performed. The desired amount of time can be in the range from about 1 hour to about 2 months, preferably about 5 to about 10 days. There are several factors that can affect the rate of dissolution of the first material **51**. According to an embodiment, the first material **51** and the second material **52** are selected such that the at least a portion of the first material **51** dissolves in the desired amount of time. By way of example, the greater the difference between the second material's anodic index and the first material's anodic index, the faster the rate of dissolution. By contrast, the less the difference between the second material's anodic index and the first material's anodic index, the slower the rate of dissolution.

By way of yet another example, the farther apart the first material and the second material are from each other in a galvanic series, the faster the rate of dissolution; and the closer together the first and second material are to each other in the galvanic series, the slower the rate of dissolution. By evaluating the difference in the anodic index of the first and second materials, or by evaluating the order in a galvanic series, one of ordinary skill in the art will be able to determine the rate of dissolution of the first material in a given electrolyte.

Another factor that can affect the rate of dissolution of the first material **51** is the proximity of the first material **51** to the second material **52**. A more detailed discussion regarding different embodiments of the proximity of the first and second materials is presented below. Generally, the closer the first material **51** is physically to the second material **52**, the faster the rate of dissolution of the first material **51**. By contrast, generally, the farther apart the first and second materials are from one another, the slower the rate of dissolution. It should be noted that the distance between the first material **51** and the second material **52** should not be so great that an electrically conductive path ceases to exist between the first and second materials. According to an embodiment, any distance between the first and second materials **51/52** is selected such that the at least a portion of the first material **51** dissolves in the desired amount of time.

Another factor that can affect the rate of dissolution of the first material **51** is the concentration of the electrolyte and the temperature of the electrolyte. A more detailed discussion of the electrolyte is presented below. Generally, the higher the concentration of the electrolyte, the faster the rate of dissolution of the first material **51**, and the lower the concentration of the electrolyte, the slower the rate of dissolution. Moreover, the higher the temperature of the electrolyte, the faster the rate of dissolution of the first material **51**, and the lower the temperature of the electrolyte, the slower the rate of dissolution. One of ordinary skill in the art can select: the exact metals and/or metal alloys, the proximity of the first and second materials, and the concentration of the electrolyte based on an anticipated temperature in order for the at least a portion of the first material **51** to dissolve in the desired amount of time.

FIG. 2 depicts the isolation device **30** according to certain embodiments. According to this embodiment, the first material **51** forms a matrix of the portion of the wellbore device that contains the first material **51** and the second material **52**. It is to be understood that the entire isolation device, for example, when the isolation device is a ball or ball seat, can be made of at least the first material and second material. Moreover, only one or more portions of the isolation device can be made from at least the first and second materials. As can be seen in FIG. 2, the second material **52** can be in the form of pieces, wherein the pieces of the second material are embedded within the matrix of the first material **51**. The exact number or concentration of the pieces of the second material **52** can be selected and adjusted to control the dissolution rate of the first material **51** such that at least the portion of the first material **51** dissolves in the desired amount of time. For example, the higher the concentration of pieces of second material **52** that are embedded within the matrix of the first material **51**, generally the faster the rate of dissolution. Moreover, the pieces of the second material **52** can be uniformly distributed throughout the matrix of the first material **51**. This embodiment can be useful when a constant rate of dissolution of the first material is desired. The pieces of the second material can also be non-uniformly distributed throughout the matrix of the first material such

that different concentrations of the second material are located within different areas of the matrix. By way of example, a higher concentration of the pieces of the second material can be distributed closer to the outside of the matrix for allowing an initially faster rate of dissolution; whereas a lower concentration of the pieces can be distributed in the middle and inside of the matrix for allowing a slower rate of dissolution. By contrast, a higher concentration of the pieces of the second material can be distributed in the middle and/or inside of the matrix for allowing a faster rate of dissolution at the end of dissolution; whereas a lower concentration of the pieces can be distributed closer to the outside of the matrix for allowing an initially slower rate of dissolution. Of course the concentration of pieces of the second material can be distributed in a variety of ways to allow for differing rates of dissolution of the first material matrix.

According to an embodiment, a third material is included in the portion of the isolation device (not shown in FIG. 2). The third material can be a bonding agent for bonding the pieces of the second material into the matrix of the first material **51**. This embodiment can be useful during the manufacturing process to provide a suitable bond between the matrix of the first material **51** and pieces of the second material **52**. Preferred manufacturing processes can include casting, forging, hot- and/or cold-working, metal injection molding, but would exclude powder compaction and sintering. Preferably, the portion of the isolation device is made via casting. Preferably, the portion of the isolation device is also modified with a heat treatment. In one embodiment, the heat treatment involves precipitation heat treatment where the alloy is heated to allow the precipitation of the constituent ingredients that are held in a solid solution. The precipitation heat treatment temperature can be in the range from 300° F. to 500° F. (149° C. to 260° C.) for 1 to 16 hours. For example, a forged metal alloy can be heated for 24 hours at 350° F. (177° C.). In another example, cast parts are heated for 1 to 2 hours at 400° F. to 500° F. (204° C. to 260° C.), followed by slow cooling. The precipitation heat treatment could follow a solution heat treatment. A solution heat treatment involves heating the metal alloy to a temperature at which certain ingredients of the alloy go into solution, and then quenching so as to hold these ingredients in solution during cooling. The solution heat treatment temperature can be in the range from 650° F. to 1050° F. (343° C. to 566° C.) for 10 to 24 hours.

Examples of materials suitable for use as a bonding third material include, but are not limited to, copper, platinum, gold, silver, nickel, iron, chromium, molybdenum, tungsten, stainless steel, zirconium, titanium, indium, and oxides of any of the foregoing. Preferably, the third material includes a metal and/or a non-metal that is different from the metals making up the first and second materials **51/52**. In one example, the first material is aluminum, the second material is iron, and the third material is iron oxide. In another example, the first material is magnesium, the second material is carbon, and the third material is iron oxide. It may be desirable to use the oxide of the metal to create a better bond between the first and second materials **51/52**. The third material can be coated onto the pieces of the second material **52**. A layer of the third material can be located between the surfaces of the pieces of the second material and the matrix of the first material with the surfaces of pieces of the second material being physically separated from the matrix of the first material via the layer of third material. The coating of third material can form a metal or metal oxide interface with the surface of each of the pieces of the second material **52**.

## 11

with the matrix of the first material **51**. Accordingly, after manufacture, there will be a layer of the third material **53** located between the surfaces of the pieces of the second material **52** and the matrix of the first material **51**. The thickness of the layer of the third material can be selected to provide the desired bond strength between the pieces of the second material **52** and matrix of the first material **51**. For example, if the layer is too thin, then there may be an insufficient amount of third material to create a good bond, and if the layer is too thick, then the layer may become mechanically weak and mechanical failure can occur at the interface between the third material **53** and the first or second materials or failure could also occur within the layer of third material. Preferably, the thickness of the layer of third material is in the range of about 10 nanometers to about 100 nanometers. In another embodiment, the thickness of the third material is less than 10 nanometers. In another embodiment, the thickness of the third material is 100 nanometers to 5,000 nanometers.

FIG. 3 depicts the isolation device according to certain other embodiments. As depicted in FIG. 3, the isolation device can comprise pieces of the first material **51**, pieces of the second material **52**, and the third material **53**. Although this embodiment depicted in FIG. 3 illustrates the isolation device as a ball, it is to be understood that this embodiment and discussion thereof is equally applicable to an isolation device that is a bridge plug, packer, etc. In order for galvanic corrosion to occur (and hence dissolution of at least a portion of the first material **51**), both, the first and second materials **51/52** need to be capable of being contacted by the electrolyte. Preferably, at least a portion of one or more pieces of the first material **51** and the second material **52** form the outside of the isolation device, such as a ball **30**. In this manner, at least a portion of the first and second materials **51/52** are capable of being contacted with the electrolyte.

FIG. 4 illustrates an example of the first material **51**, the second material **52**, and the third material **53** according to certain other embodiments. As depicted in FIG. 4, the third material **53** is a bonding agent for bonding the pieces of the first material **51** and second material **52** together.

FIG. 5 illustrates an example of the first material **51**, the second material **52**, and the third material **53** according to certain other embodiments. As depicted in FIG. 5, the third material **53** is coated onto the pieces of the first material **51** and second material **52**. In some further examples, the third material **53** which was coated onto the pieces of the first material **51** and second material **52** may also bond the pieces of the first **51** and second material **52** together.

FIG. 6 illustrates an example of the first material **51**, the second material **52**, and the third material **53** according to certain other embodiments. As depicted in FIG. 6, the third material **53** is a bonding agent for bonding the pieces of the second material **52** into the matrix of the first material **51**.

According to another embodiment, the third material **53** physically separates at least a portion of a surface of one or more pieces of the first material **51** from at least a portion of a surface of one or more pieces of the second material **52**. These embodiments can be useful when it is desired to use the distance between the first and second materials **51/52** as a way to control the rate of dissolution of the first material **51**. The third material **53** may also limit the ionic conductivity or the electrical conductivity between the first and second materials **51/52**. According to an embodiment, the third material **53** is in the form of pieces. The third material can be selected from the group consisting of metals, non-metals, sand, plastics, ceramics, and polymers. Preferably, the third material includes a metal and/or a non-metal that is

## 12

different from the metals making up the first and second materials **51/52**. The pieces of the third material **53** can be located between one or more of the pieces of the first and second materials **51/52**. The size and shape of the pieces of the third material **53** can be selected to provide a desired distance of the physical separation of the first and second materials **51/52**. By way of example, the thicker the cross-sectional size of the piece of third material **53**, the greater the reduction of the ionic and/or electrical conductivity between the pieces of the first material **51** and the pieces of the second material **52**. Conversely, the smaller the thickness of the third material, the smaller the reduction of the ionic and/or electrical conductivity between the pieces of the first and second materials **51/52**. The pieces of the third material **53** can also separate two or more pieces of the first material **51** and/or two or more pieces of the second material **52**. The size of the pieces of the third material **53** can be the same or different. The pieces of third material having different thicknesses can be distributed throughout the portion of the isolation device in a variety of ways to provide different rates of dissolution. For example, larger-sized pieces can be located towards the outside of the portion of the isolation device; whereas smaller-sized pieces can be located towards the middle and/or inside. This embodiment could provide an initially slower rate of dissolution due to the initially greater distance between the first and second materials **51/52** and a faster rate of dissolution later due to a decreased distance between the first and second materials **51/52**. Of course, the distribution of different sized pieces of the third material **53** can vary and be selected to provide the desired rates of dissolution of at least some of the pieces of the first material **51**.

The concentration and distribution patterns of pieces of the third material **53** can also be selected to provide the desired rate of dissolution of at least some of the pieces of the first material **51** such that at least some of the pieces of the first material dissolve in the desired amount of time. For example, generally, the higher the concentration of the third material, the slower the rate of dissolution, and the lower the concentration of the third material, the faster the rate of dissolution. Moreover, the pieces of the third material **53** can be uniformly distributed throughout the portion of the isolation device containing the first, second, and third materials. This embodiment (assuming a relatively uniform size of the pieces of third material) can be used to provide a relatively constant rate of dissolution of the pieces of the first material **51**. The pieces of the third material **53** can also be non-uniformly distributed throughout the portion of the isolation device. By way of example, a higher concentration of the pieces of the third material can be distributed closer to the outside of the portion of the isolation device for allowing an initially slower rate of dissolution; whereas a lower concentration of the pieces can be distributed in the middle and inside for allowing a faster rate of dissolution. By contrast, a higher concentration of the pieces of the third material can be distributed in the middle and/or inside of the matrix for allowing a slower rate of dissolution at the end of dissolution; whereas a lower concentration of the pieces can be distributed closer to the outside for allowing an initially faster rate of dissolution.

The pieces of the first material **51** and the pieces of the second material **52** can be bonded together via a third material as described above with reference to FIG. 2. In this manner, the pieces of first material and pieces of the second material can be bonded together to form the portion of the

isolation device. The device of FIG. 3 can also be manufactured and optionally subjected to the heat treatments described above.

The size, shape and placement of the pieces of the first and second materials 51/52 can also be adjusted to control the rate of dissolution of the first material 51. By way of example, generally the smaller the cross-sectional area of each piece, the faster the rate of dissolution. The smaller cross-sectional area increases the ratio of the surface area to total volume of the material, thus allowing more of the material to come in contact with the electrolyte. The cross-sectional area of each piece of the first material 51 can be the same or different, the cross-sectional area of each piece of the second material 52 can be the same or different, and the cross-sectional area of the pieces of the first material 51 and the pieces of the second material 52 can be the same or different. Additionally, the cross-sectional area of the pieces forming the outer portion of the isolation device and the pieces forming the inner portion of the isolation device can be the same or different. By way of example, if it is desired for the outer portion of the isolation device to proceed at a faster rate of galvanic corrosion compared to the inner portion of the device, then the cross-sectional area of the individual pieces comprising the outer portion can be smaller compared to the cross-sectional area of the pieces comprising the inner portion. The shape of the pieces of the first and second materials 51/52 can also be adjusted to allow for a greater or smaller cross-sectional area.

According to an embodiment, at least the first material 51 and second material 52 are capable of withstanding a specific pressure differential for a desired amount of time. As used herein, the term “withstanding” means that the substance does not crack, break, or collapse. The pressure differential can be the downhole pressure of the subterranean formation 20 across the device. As used herein, the term “downhole” means the location of the wellbore where the portion of the isolation device is located. Formation pressures can range from about 1,000 to about 30,000 pounds force per square inch (psi) (about 6.9 to about 206.8 megapascals (“MPa”). The pressure differential can also be created during oil or gas operations. For example, a fluid, when introduced into the wellbore 11 upstream or downstream of the substance, can create a higher pressure above or below, respectively, of the isolation device. Pressure differentials can range from 100 to over 10,000 psi (about 0.7 to over 68.9 MPa). According to another embodiment, the isolation device is capable of withstanding the specific pressure differential for the desired amount of time. The desired amount of time can be at least 30 minutes. The desired amount of time can also be in the range of about 30 minutes to 14 days, preferably 30 minutes to 2 days, more preferably 4 hours to 24 hours.

As discussed above, the rate of dissolution of the first material 51 can be controlled using a variety of factors. According to an embodiment, at least the first material 51 includes one or more tracers (not shown). The tracer(s) can be, without limitation, radioactive, chemical, electronic, or acoustic. As depicted in FIG. 3, each piece of the first material 51 can include a tracer. A tracer can be useful in determining real-time information on the rate of dissolution of the first material 51. For example, a first material 51 containing a tracer, upon dissolution can be flowed through the wellbore 11 and towards the wellhead or into the subterranean formation 20. By being able to monitor the presence of the tracer, workers at the surface can make on-the-fly decisions that can affect the rate of dissolution of the remaining first material 51.

Such decisions might include to increase or decrease the concentration of the electrolyte. As used herein, an electrolyte is any substance containing free ions (i.e., a positive- or negative-electrically charged atom or group of atoms) that make the substance electrically conductive. The electrolyte can be selected from the group consisting of, solutions of an acid, a base, a salt, and combinations thereof. A salt can be dissolved in water, for example, to create a salt solution. Common free ions in an electrolyte include sodium ( $Na^+$ ), 10 potassium ( $K^+$ ), calcium ( $Ca^{2+}$ ), magnesium ( $Mg^{2+}$ ), chloride ( $Cl^-$ ), hydrogen phosphate ( $HPO_4^{2-}$ ), and hydrogen carbonate ( $HCO_3^-$ ). The concentration (i.e., the total number of free ions available in the electrolyte) of the electrolyte can be adjusted to control the rate of dissolution of the first 15 material 51. According to an embodiment, the concentration of the electrolyte is selected such that the at least a portion of the first material 51 dissolves in the desired amount of time. If more than one electrolyte is used, then the concentration of the electrolytes is selected such that the first 20 material 51 dissolves in a desired amount of time. The concentration can be determined based on at least the specific metals or metal alloys selected for the first and second materials 51/52 and the bottomhole temperature of the well. Moreover, because the free ions in the electrolyte 25 enable the electrochemical reaction to occur between the first and second materials 51/52 by donating its free ions, the number of free ions will decrease as the reaction occurs. At some point, the electrolyte may be depleted of free ions if there is any remaining first and second materials 51/52 that 30 have not reacted. If this occurs, the galvanic corrosion that causes the first material 51 to dissolve will stop. In this example, it may be necessary to cause or allow the first and second materials to come in contact with a second, third, or fourth, and so on, electrolyte(s).

It may be desirable to delay contact of the first and second materials 51/52 with the electrolyte. The isolation device can further include a coating 60 on the outside of the device. The coating can be a compound, such as a wax, thermoplastic, sugar, salt, or a conducting polymer and can include chromates, phosphates, and polyanilines. The coating can be selected such that the coating dissolves in wellbore fluids, melts at a certain temperatures, or cracks and falls away. Upon dissolution or melting, at least the first material 51 of the isolation device is available to come in contact with the electrolyte. The coating 60 can also be porous to allow the electrolyte to come in contact with some of the surface of the first and second materials 51/52.

It may also be desirable to selectively dissolve certain portions of the first material 51 at different times or at different rates. By way of example, it may be desirable to dissolve the top portion of the isolation device first and then dissolve the bottom portion at a later time. This can be accomplished, for example, by introducing a first electrolyte into the wellbore to come in contact with the first and second materials 51/52. There are many operations, such as stimulation operations involving fracturing or acidizing techniques, or tertiary recovery operations involving injection techniques, in which this may be desirable. After the desired operation has been performed, the bottom of the isolation device can be contacted by produced formation fluids. The formation fluids can contain a sufficient concentration of free ions to allow the dissolution of the remaining first material 51.

The methods include the step of contacting or allowing the wellbore isolation device to come in contact with the electrolyte. The step of contacting can include introducing the electrolyte into the wellbore 11. The step of allowing can

## 15

include allowing the isolation device to come in contact with a fluid, such as a reservoir fluid. The methods can include contacting or allowing the device to come in contact with two or more electrolytes. If more than one electrolyte is used, the free ions in each electrolyte can be the same or different. A first electrolyte can be, for example, a stronger electrolyte compared to a second electrolyte. Furthermore, the concentration of each electrolyte can be the same or different. It is to be understood that when discussing the concentration of an electrolyte, it is meant to be a concentration prior to contact with either the first and second materials 51/52, as the concentration will decrease during the galvanic corrosion reaction. Tracers can be used to help determine the necessary concentration of the electrolyte to help control the rate and finality of dissolution of the first material 51. For example, if it is desired that the first material 51 dissolves to a point to enable the isolation device to be flowed from the wellbore 11 within 5 days and information from a tracer indicates that the rate of dissolution is too slow, then a more concentrated electrolyte can be introduced into the wellbore or allowed to contact the first and second materials 51/52. By contrast, if the rate of dissolution is occurring too quickly, then the first electrolyte can be flushed from the wellbore and a less concentrated electrolyte can then be introduced into the wellbore.

The methods can further include the step of placing the isolation device in a portion of the wellbore 11, wherein the step of placing is performed prior to the step of contacting or allowing the isolation device to come in contact with the electrolyte. More than one isolation device can also be placed in multiple portions of the wellbore. The methods can further include the step of removing all or a portion of the dissolved first material 51 and/or all or a portion of the second material 52 or the substance 60, wherein the step of removing is performed after the step of allowing the at least a portion of the first material to dissolve. The step of removing can include flowing the dissolved first material 51 and/or the second material 52 or substance 60 from the wellbore 11. According to an embodiment, a sufficient amount of the first material 51 dissolves such that the isolation device is capable of being flowed from the wellbore 11. According to this embodiment, the isolation device should be capable of being flowed from the wellbore via dissolution of the first material 51, without the use of a milling apparatus, retrieval apparatus, or other such apparatus commonly used to remove isolation devices. According to an embodiment, after dissolution of the first material 51, the second material 52 or the substance 60 has a cross-sectional area less than 0.05 square inches, preferably less than 0.01 square inches.

Therefore, the present invention is well adapted to attain the ends and advantages mentioned as well as those that are inherent therein. The particular embodiments disclosed above are illustrative only, as the present invention may be modified and practiced in different but equivalent manners apparent to those skilled in the art having the benefit of the teachings herein. Furthermore, no limitations are intended to the details of construction or design herein shown, other than as described in the claims below. It is, therefore, evident that the particular illustrative embodiments disclosed above may be altered or modified and all such variations are considered within the scope and spirit of the present invention. While compositions and methods are described in terms of "comprising," "containing," or "including" various components or steps, the compositions and methods also can "consist essentially of" or "consist of" the various components and steps. Whenever a numerical range with a lower limit and an

## 16

upper limit is disclosed, any number and any included range falling within the range is specifically disclosed. In particular, every range of values (of the form, "from about a to about b," or, equivalently, "from approximately a to b") disclosed herein is to be understood to set forth every number and range encompassed within the broader range of values. Also, the terms in the claims have their plain, ordinary meaning unless otherwise explicitly and clearly defined by the patentee. Moreover, the indefinite articles "a" or "an," as used in the claims, are defined herein to mean one or more than one of the element that it introduces. If there is any conflict in the usages of a word or term in this specification and one or more patent(s) or other documents that may be incorporated herein by reference, the definitions that are consistent with this specification should be adopted.

What is claimed is:

1. A method of removing a wellbore isolation device comprising: contacting or allowing the wellbore isolation device to come in contact with an electrolyte, wherein the wellbore isolation device is produced by casting, and wherein the wellbore isolation device is not produced by powdered compaction and sintering, wherein at least a portion of the wellbore isolation device comprises a first material, pieces of a second material, and a third material, wherein after the casting at least one of the first material, the second material and the third material is heated to go into solution, and wherein the first material: (A) is a metal or a metal alloy; (B) forms a matrix of the portion of the wellbore isolation device; and (C) partially or wholly dissolves when an electrically conductive path exists between the first material and the second material and at least a portion of the first and second materials are in contact with the electrolyte, wherein the pieces of the second material: (A) are a metal or metal alloy; and (B) are embedded within the matrix of the first material; wherein the first material and the second material form a galvanic couple and wherein the first material is the anode and the second material is the cathode of the couple; and wherein the third material is a bonding agent for bonding the pieces of the second material into the matrix of the first material, allowing at least a portion of the first material to dissolve.

2. The method according to claim 1, wherein the isolation device is capable of restricting or preventing fluid flow between a first wellbore interval and a second wellbore interval.

3. The method according to claim 1, wherein isolation device is a ball and a seat, a plug, a bridge plug, a wiper plug, a packer, or a plug for a base pipe.

4. The method according to claim 1, wherein the metal or metal alloy of the first material and the second material are selected from the group consisting of, magnesium, aluminum, zinc beryllium, tin, iron, nickel, copper, oxides of any of the foregoing, and combinations thereof.

5. The method according to claim 1, wherein at least the portion of the first material dissolves in a desired amount of time.

6. The method according to claim 5, wherein the metals or metal alloys of the first material and the second material are selected such that the at least a portion of the first material dissolves in the desired amount of time.

7. The method according to claim 5, wherein the concentration of the electrolyte is selected such that the at least a portion of the first material dissolves in the desired amount of time.

8. The method according to claim 5, wherein the concentration of the pieces of the second material is selected to

## 17

control the dissolution rate of the first material such that at least the portion of the first material dissolves in the desired amount of time.

9. The method according to claim 1, wherein the pieces of the second material are uniformly distributed throughout the matrix of the first material. 5

10. The method according to claim 1, wherein the pieces of the second material are non-uniformly distributed throughout the matrix of the first material such that different concentrations of the second material are located within 10 different areas of the matrix.

11. The method according to claim 1, wherein the third material is selected from the group consisting of copper, platinum, gold, silver, nickel, iron, chromium, molybdenum, tungsten, stainless steel, zirconium, titanium, indium, oxides 15 of any of the foregoing, and any combinations thereof.

12. The method according to claim 1, wherein the third material is coated onto the pieces of the second material.

13. The method according to claim 12, wherein a layer of 20 the third material is located between the surfaces of the pieces of the second material and the matrix of the first material with the surfaces of pieces of the second material being physically separated from the matrix of the first material via the layer of third material.

14. The method according to claim 13, wherein the thickness of the layer of the third material is selected to provide a desired bond strength between the pieces of the second material and the matrix of the first material. 25

15. The method according to claim 1, further comprising the step of placing the isolation device into a portion of the wellbore, wherein the step of placing is performed prior to the step of contacting or allowing the isolation device to come in contact with the electrolyte. 30

16. The method according to claim 1, wherein the third material physically separates at least a portion of a surface of one or more pieces of the first material from at least a portion of a surface of one or more pieces of the second material, wherein the third material is a bonding agent for bonding the pieces of the first and second materials together. 35

17. A method of removing a wellbore isolation device comprising:

contacting or allowing the wellbore isolation device to come in contact with an electrolyte, wherein at least a 40

## 18

portion of the wellbore isolation device comprises pieces of a first material, pieces of a second material, and a third material, wherein the first material:

(A) is a metal or a metal alloy; and  
(B) partially or wholly dissolves when an electrically

conductive path exists between the first material and the second material and at least a portion of the first and second materials are in contact with the electrolyte,

wherein the second material is a metal or metal alloy, wherein the first material and the second material form a galvanic couple and wherein the first material is the anode and the second material is the cathode of the couple, and

wherein the third material physically separates at least a portion of a surface of one or more pieces of the first material from at least a portion of a surface of one or more pieces of the second material, wherein the third material is a bonding agent for bonding the pieces of the first and second materials together; and allowing at least some of the pieces of the first material to dissolve.

18. The method according to claim 17, wherein the concentration and distribution pattern of the third material is selected to provide a desired rate of dissolution of at least some of the pieces of the first material such that at least some of the pieces of the first material dissolve in a desired amount of time.

19. The method according to claim 17, wherein the third material is coated onto the pieces of the first and second materials.

20. The method according to claim 19, wherein a layer of the third material is located between the surfaces of the pieces of the first and second materials with the surfaces of pieces of the first material being physically separated from the surfaces of pieces of the second material via the layer of third material.

21. The method according to claim 20, wherein the thickness of the layer of the third material is selected to provide a desired bond strength between the pieces of the first and second materials.

\* \* \* \* \*